

# United States Patent Office

2,955,036

Patented Oct. 4, 1960

1

2,955,036

## FOG REDUCTION IN PHOTOGRAPHIC SILVER HALIDE EMULSIONS

Fritz Dersch and Millet R. De Angelus, Binghamton, N.Y., assignors to General Aniline & Film Corporation, New York, N.Y., a corporation of Delaware

No Drawing. Filed Apr. 25, 1958, Ser. No. 730,794

8 Claims. (Cl. 96—66)

The present invention relates to the use of antifogging and stabilizing agents for photographic silver halide emulsions and, more particularly, to the employment of S-carboxy-alkyl-cysteines, their salts and esters for such purpose.

It is recognized that light sensitive emulsions such as gelatino silver halide emulsions have a tendency to fog. The fog may be caused in a number of ways as, for example, by excessive ripening of the emulsion, by storage of the light sensitive element at elevated temperatures and humidity, or by prolonged development of the exposed emulsion.

A great number of antifogging and stabilizing agents have been recommended in the literature for the purpose of preventing the formation of fog in light sensitive silver halide emulsions. Although these compounds have the ability to control fog during manufacture, as well as during storage, they also have distinct shortcomings. For instance, they lower the sensitivity of the emulsion either immediately or under storage conditions, thus causing speed regression.

We have now found that the S-carboxyalkyl-cysteines, their salts and esters are excellent stabilizers and antifogging agents for silver halide emulsions having the ability to maintain the sensitivity and fog at or close to initial optimum values under keeping conditions of high temperature and humidity.

The use of such compounds to inhibit fog and to stabilize silver halide emulsions either by location of the same in the emulsion, in layers adjacent to the emulsion or in processing baths for the emulsion constitutes the purposes and objects of the present invention.

The S-carboxy-(lower)-alkyl-cysteines, the use of which is contemplated herein, may be represented by the following formula:



wherein R is hydrogen, an aliphatic radical such as lower alkyl, i.e. methyl, ethyl, propyl, butyl, amyl and the like; hydroxylalkyl, i.e., hydroxymethyl, hydroxyethyl and the like; carboxylalkyl, i.e., carboxymethyl, carboxyethyl and the like; aryl such as phenyl, toluyl, naphthyl, and the like; aralkyl such as benzyl, phenethyl and the like; or a salt forming group, i.e., sodium, potassium, ammonium, silver, triethylamine, diethylamine, triethanolamine and the like; R<sub>1</sub> is a hydrogen atom, an acyl radical, i.e., acetyl, propenyl, butyryl, benzoyl, phenacyl, and the like; and n is a whole number of from 1 to 3.

Examples of compounds within the ambit of such a formula which we have found to be effective are:



S-carboxymethylcysteine and its sodium, potassium, ammonium, silver or organic amine salts.



2

S-( $\beta$ -carboxyethyl)-cysteine and its sodium, potassium, ammonium, silver or amine salt.

S-( $\gamma$ -carboxypropyl)-cysteine and the methyl, ethyl or phenyl esters thereof.

S-carboxymethyl-cysteine hydrochloride



S-carboxymethyl-cysteine ethyl ester

S-( $\beta$ -carboxymethyl)-cysteine ethyl ester



N-benzoyl-S-carboxymethyl-cysteine



N-benzoyl-S-carboxymethyl-cysteine methyl ester.

N-benzoyl-S-carboethoxymethyl-cysteine ethyl ester.

N-acetyl-S-carboxymethyl-cysteine ethyl ester. The above compounds are best prepared by reacting in aqueous solution and in a mildly alkaline medium (pH=8.0-9.0) cysteine hydrochloride with a halogeno aliphatic acid such as chloroacetic acid, bromoacetic acid, iodoacetic acid,  $\beta$ -bromopropionic acid or  $\gamma$ -bromobutyric acid in the presence of an acid binding agent such as sodium hydroxide, potassium hydroxide or the like. After standing for several hours, the S-carboxyalkyl-cysteine precipitates from the reaction mixture. Alternatively, the

S-carboxyalkyl-cysteine can also be prepared according to the procedures described in J. Biol. Chem. Soc., vol. 106, pages 331-341; J.A.C.S., vol. 66, pages 1757-9, and Helv. Chim. Acta, vol. 27, pages 1280-4.

The S-carboxyalkyl-cysteine thus formed may be converted to its salt by reacting it with a water soluble alkali compound containing the desired cation such as potassium carbonate, sodium carbonate, ammonium carbonate or the like or with a suitable acid such as hydrochloric acid, hydrobromic acid and the like.

If the esters are desired, they may be produced in the conventional manner by refluxing the free acid with the desired alcohol such as methyl alcohol, ethyl alcohol, butyl alcohol or with a phenol in the presence of hydrochloric acid. The diesters are prepared by reacting cysteine with the ester of a halogen substituted aliphatic acid followed by treatment with an alcohol in an acid medium to insure complete esterification.

Beneficial effects and fog reduction are obtained when aqueous or alcoholic solutions of the aforementioned compounds are incorporated in the silver halide emulsions as "ripening finals" or as "coating finals." "Ripening finals" are added during the ripening or the sensitivity increasing stage of the emulsion making process. Such additions may be made before, during or after the decomposition of the soluble silver salt such as silver nitrate by means of a soluble halide such as potassium bromide, sodium chloride or the like in the presence of a colloidal carrier such as gelatin, PVA, solubilized casein or albumen.

"Coating finals" are added to the emulsion just prior to coating on a suitable support such as glass, paper or film at a time when the emulsion has nearly obtained its maximum sensitivity.

When used as ripening finals, the antifogging agents are best employed in a concentration of 0.20 to 2.5 milligrams per mol of silver halide and when used as coating finals in a concentration of 0.2 to 10 milligrams per mol of silver halide. The concentration used depends on the type of emulsion employed, and it is advisable to determine the optimum concentration from case to case. In some instances, it is advantageous to apply the anti-

fogant and stabilizers in layers adjacent to the emulsion, that is, in a separate undercoating layer or in the anti-abrasion gelatin surface. In other instances, the desired result may be obtained by addition of the anti-fogant and stabilizer to one or several processing baths such as developer, prebath or the like.

The aforesaid antifoggants and stabilizers may be utilized in connection with any type of photographic emulsion, e.g., non-sensitized, orthochromatic, panchromatic, boil type emulsions, ammonia type emulsions, X-ray emulsions, paper emulsions, color emulsions or the like. They may be employed in combination with other known antifoggants and stabilizers, reduction- and metal- and noble metal sensitizers, or in combination with hydroxy-polyethenoxy derivates, i.e., those obtained by reacting ethylene oxide with an alcohol, phenol, amine or the like (see U.S. Patent 1,970,578).

Although our stabilizers are somewhat related to cysteine, cystine and methionine which were previously recommended as emulsion additives, these compounds provide even under optimum conditions only a limited antifogging protection. These moderate benefits are accompanied by a number of undesirable properties, such as reduced sensitivity of the emulsion and lowered contrast together with increased fog under conditions of high-temperature storage. The compounds of our invention are free from these disadvantages.

The invention is illustrated by the following examples, but it is to be understood that the invention is not restricted thereto.

#### Example I

A silver halide emulsion in gelatin containing 4 percent silver iodide and 96 percent silver bromide was prepared in a conventional manner and brought up to its maximum light sensitivity. It was then readied for coating, finals were added such as sensitizing dyes, stabilizers and hardening agents. A 1 percent solution of S-( $\beta$ -carboxyethyl)-cysteine was added to the emulsion as an antifogant. The emulsion samples weighed one kilogram and contained about .4 mol of silver halide. The so prepared emulsion samples were coated on a suitable cellulose ester base and dried. Samples of these film coatings were then exposed in a Type IIB Sensitometer and developed in a developer of the following composition:

|                                     | Grams |
|-------------------------------------|-------|
| Metol (p-methylaminophenol sulfate) | 1.5   |
| Sodium sulfite, anhydrous           | 45    |
| Sodium bisulfite                    | 1     |
| Hydroquinone                        | 3     |
| Sodium carbonate, monohydrated      | 6     |
| Potassium bromide                   | 0.8   |
| Water to make 1 liter.              |       |

| Quantity of Compound added | Relative Speed | Fog at 6' Dev. | Speed after oven test | Oven fog at 6' Development |
|----------------------------|----------------|----------------|-----------------------|----------------------------|
| 0                          | 100            | .16            | 85                    | .54                        |
| 1 mg.                      | 100            | .14            | 100                   | .40                        |
| 4 mg.                      | 100            | .12            | 120                   | .28                        |

The S-( $\beta$ -carboxyethyl)-cysteine was prepared as follows:

15.7 grams cysteine hydrochloride (0.1 mol) was added to 100 milliliters of 1.0 N sodium hydroxide solution and the pH adjusted to a point between 8 and 9. To this dispersion was added a solution of 15.3 grams of  $\beta$ -bromo-propionic acid in 50 milliliters of water whereupon the pH dropped to 6. Additional small increment of 1.0 N sodium hydroxide was added gradually so that the solution was slightly alkaline at all times. After 15 hours' standing, a white precipitate formed which was filtered off. The yield was improved by acidifying the filtrate with 6.0 N hydrochloric acid under cooling. The

65  
70  
75

precipitates were combined and purified by recrystallization from water. The product melted at 192° C. The product had the following formula:



An analysis gave the following results:

|                 | C     | H    | N    | S     |
|-----------------|-------|------|------|-------|
| Calculated..... | 33.52 | 5.03 | 7.82 | 17.88 |
| Found.....      | 33.24 | 5.24 | 7.68 | 17.51 |

#### Example II

The procedure was the same as in Example I excepting that the S-( $\beta$ -carboxyethyl)-cysteine was replaced by an equivalent quantity of S-carboxymethylcysteine. Results similar to those obtained in Example I were secured in this instance.

This compound was prepared by reacting cysteine with chloroacetic acid as described in J.A.C.S., vol. 66, page 1758.

#### Example III

The procedure was the same as in Example I except that the S-( $\beta$ -carboxyethyl)-cysteine was replaced by an equivalent quantity of N-acetyl-S-carbethoxymethylcysteine ethyl ester. The results were similar to those of Example I. This product was prepared according to the procedure described in Helv. Chim. Acta, vol. 27, pages 1280-4, by reacting cysteine hydrochloride in an alkaline medium successively with chloroacetic acid and acetic anhydride and esterifying the resultant dicarboxylic acid.

#### Example IV

The procedure was the same as in Example I excepting that the S-( $\beta$ -carboxyethyl)-cysteine was replaced by an equivalent quantity of N-acetyl-S-( $\beta$ -carboxyethyl)-cysteine. The results were similar to those obtained in Example I.

#### Example V

The antifogging action of S-( $\beta$ -carboxyethyl)-cysteine was compared with that of cysteine and cystine. The following results were obtained.

| Quantity of Compound                      | Shortly after coating |                       | After incubation |                      |
|-------------------------------------------|-----------------------|-----------------------|------------------|----------------------|
|                                           | Relative Speed        | Fog at 12' Developing | Relative Speed   | Fog at 6' Developing |
| 5 mg. S-( $\beta$ -carboxyethyl)-cysteine | 100                   | .27                   | 100              | .14                  |
| 5 mg. cystine                             | 75                    | .29                   | 50               | .16                  |
| 5 mg. cysteine                            | 110                   | .54                   | 80               | .40                  |
| Type                                      | 100                   | .27                   | 100              | .18                  |

It is evident from this table that the S-( $\beta$ -carboxyethyl)-cysteine reduces fog without loss of speed to a greater extent than the cysteine and the cystine which, in addition to their poorer antifogging performance, cause a serious loss of speed.

#### Example VI

A gelatin solution containing 30 grams of gelatin, 100 mg. of S-( $\beta$ -carboxyethyl)-cysteine per liter was coated on filmbase in a manner known to the art. After the coating was performed, a silver halide emulsion in gelatin containing 4 percent of silver iodide and 96 percent of silver bromide was coated on top of the previously coated gelatin layer. After drying, film samples were exposed and processed as described in Example III. The samples exhibited a relative speed of 100 and a fog of 0.12 compared with a type coating of the same emulsion having an undercoating similar to that described above, but

lacking the antifoggant and having a speed of 100 and a fog of 0.20.

*Example VII*

Exposed samples of a photographic film were developed for twelve minutes at 65° F. in a standard metol-hydroquinone developer. Two tests were made, one with the normal developing solution and one with a developer containing 10 mgs. of S-( $\beta$ -carboxyethyl)-cysteine per liter of developer. Sensitometric strips, developed in the normal developer (control) for twelve minutes, showed a fog of .30, whereas those strips which were developed in the developer containing the antifoggant had a fog of .20.

Various modifications of the invention will occur to persons skilled in the art. Thus, it is understood that in lieu of using the particular antifoggants of the examples, any of the antifoggants listed in the application may be employed with equivalent results. We, therefore, do not intend to be limited in the patent granted except as necessitated by the prior art and the appended claims.

We claim:

1. A light sensitive photographic material comprising a base and a light sensitive silver halide emulsion, said light sensitive material containing as an antifoggant a compound of the following constitution:



wherein R is selected from the class consisting of hydrogen, and alkyl, hydroxyalkyl, carboxyalkyl, aryl and aralkyl radical and a sodium, potassium, ammonium, silver and an amine cation; R<sub>1</sub> is a member selected from the class consisting of hydrogen and acyl groups wherein the total number of carbon atoms in said radicals and groups does not exceed eight; and n is a whole number ranging from 1 to 3.

2. The article as defined in claim 1 wherein the antifoggant is located in the silver halide emulsion.

3. The article as defined in claim 1 wherein the anti-

foggant is located in a layer adjacent to said silver halide emulsion layer.

4. A light sensitive photographic material comprising a base with a light sensitive silver halide emulsion thereon, said emulsion containing as an antifoggant the compound S-( $\beta$ -carboxyethyl)-cysteine.

5. A light sensitive photographic material comprising a base with a light sensitive silver halide emulsion thereon, said emulsion containing as an antifoggant the compound S-(carboxymethyl)-cysteine.

10 6. The process of minimizing and preventing fog in light sensitive silver halide materials comprising a base having a light sensitive silver halide emulsion thereon, which comprises exposing said emulsion to light and 15 developing the same in the presence of an antifoggant having the following structural formula:



20 25 wherein R is selected from the class consisting of hydrogen, an alkyl, hydroxyalkyl, carboxyalkyl, aryl and aralkyl radical and a sodium, potassium, ammonium, silver and an amine cation; R<sub>1</sub> is a member selected from the class consisting of hydrogen and acyl groups wherein the total number of carbon atoms in said radicals and groups does not exceed eight; and n is a whole number ranging from 1 to 3.

7. The process as defined in claim 6 wherein the antifoggant is S-( $\beta$ -carboxyethyl)-cysteine.

30 35 8. The process as defined in claim 6 wherein the antifoggant is S-carboxymethyl-cysteine.

References Cited in the file of this patent

UNITED STATES PATENTS

|           |                |                |
|-----------|----------------|----------------|
| 2,363,777 | Downing et al. | Nov. 28, 1944  |
| 2,438,716 | Mueller        | Mar. 30, 1948  |
| 2,449,153 | Urbach         | Sept. 14, 1948 |